

June 4, 1935.

T. J. HANKINS, JR

2,003,486

HEAT TREATMENT OF METALS

Filed Nov. 1, 1932



INVENTOR  
THOS. J. HANKINS, JR.  
BY *M. F. Reges*  
ATTORNEY

## UNITED STATES PATENT OFFICE

2,003,486

## HEAT TREATMENT OF METALS

Thomas J. Hankins, Jr., Springfield, N. J., assignor to Westinghouse Lamp Company, a corporation of Pennsylvania

Application November 1, 1932, Serial No. 646,621

2 Claims. (CL 219—11)

This invention relates to the heat treatment of metals and in its more specific aspect is directed to the heat treatment of a refractory metal.

In the manufacture or preparation of refractory metals, as for example tungsten wires, it is customary to first prepare tungsten powder of the desired size and purity. This powder is then placed in a die of predetermined dimensions and subjected to a pressing operation in order to convert the same from a powdered state into a bar. The so prepared bar has not much body strength but has sufficient strength so that it may be handled without falling apart.

The second stage generally comprises placing the prepared tungsten bar in a hydrogen furnace operated at a comparatively low temperature, as for example 1250 degrees centigrade. The bar is maintained in said furnace for a sufficient length of time so that the particles of tungsten comprising the bar may become at least partially sintered and any superficial oxidation of some of the tungsten particles is obviated because of this reducing atmosphere.

The third stage, which is the stage with which this invention is specifically concerned, generally comprises placing the cintered bar between a pair of terminals and passing an electric current through said bar in order to effect a complete sintering of at least most if not all of the tungsten particles comprising said bar. The voltage impressed between the terminals of this bar to be treated depends upon the size of the bar.

The magnitude of the current that passes through the bar so that the above results may be obtained depends upon the cross sectional dimensions of the bar. Following this stage the completely sintered bar is generally subjected to a mechanical operation in order to reduce the cross section thereof and simultaneously increase its length. This last operation, together with the succeeding operations and the operations noted in the first two steps of this disclosure, do not form the essence of this invention. The crux of the invention resides in the third step and it is especially concerned with the problem of contacts.

Prior to my invention it has been proposed to clamp each end of a partially sintered bar and thereafter pass an electric current therethrough in order to completely sinter the particles thereof. The main disadvantage of this process is that the ends of the bar which are surrounded by the clamp do not attain the desired temperature because of the thermal conduction

of the clamps which prevents the ends of the bar from being heated to the desired temperature essential to complete the sintering.

I have found that after a bar has been subjected to heat treatment, when clamps are employed, those portions of the bar, namely the ends which are contiguous with the clamping means are without the scope of the normal specifications. That is to say, the ends of the bar surrounded by the clamping means do not have the particles thereof completely sintered with respect to each other. The percentage of the bar so clamped is about from five to twenty-five percent of the whole depending upon the length of the bar being treated. Since these ends are without the normal specification, the bar must be cut intermediate its ends in order to eliminate those portions thereof that are not completely sintered. The tungsten may, of course, be retreated. This, however, represents a high operating loss and increases the cost of production.

One other method heretofore proposed for the same general purpose and to avoid the use of clamping means involves simply butt-ending the bar to be treated between a pair of plane contact terminals generally composed of tungsten or molybdenum. The bars that emerge from the hydrogen furnace generally are not true-ended and the contact surfaces thereof that are to be placed between and contiguous with the contact terminals are not absolutely plane and oftentimes are of a macroscopically non-planar contour. These bars when placed between the contacts and in a butt-ended position do not form a firm large surface contact between the contact terminals and the ends thereof.

Therefore, when the bar is energized by an electric current in order to heat the same, there generally prevails an appreciable degree of arcing between the contact terminals and the ends of the bar. This arcing causes excessive pitting of the bar ends and also of the contact terminals located adjacent thereto.

In addition, it is found that sometimes during this heat treatment the bar under consideration, for one reason or another, becomes distorted. The result of this distortion is that the end of the bar, which is normally contiguous with the contact terminals, lifts therefrom at one edge to cause appreciable arcing between that face and the contact terminal. When this condition exists the current density at that portion of the bar which is directly contiguous with the contact ter-

5 minal may be two or three times that at the center of the bar.

10 This abnormally high energy input at the contacting area causes the metal immediately adjacent thereto to become fused so that it may flow and coat the contact at that point. This fusion may at times form a weld at the area of contact which may necessitate breaking the bar in order that it may be removed from the contact terminal. That portion which is firmly united with the contact terminal must be ground or subjected to some other operation in order that it may be removed therefrom.

15 I have found that bars that are heat treated according to this method and even though they do not become welded to the contact terminals and may be removed therefrom, are not entirely satisfactory because of the metallic structure at these ends caused by the arcing between the contact terminals and the ends thereof. When a bar of this character is subjected to a rolling operation, the ends thereof may not be worked in the same manner as that portion of the bar intermediate said ends. This is generally evidenced 20 by an apparent "fanning" of the ends thereof. Consequently it is apparent that the ends of the bar which become fan-shaped during the rolling operation must be severed therefrom.

25 In order to obviate the difficulties inherent in the clamping as well as in the aforementioned butt-ending means during the heat treatment at the third stage as heretofore set forth, I have developed the following invention.

30 The primary object of my invention is to provide means for the elimination of the end losses which are generally inherent in the past process as heretofore set forth.

35 Another object of my invention is to provide a simple and inexpensive means for efficiently heat-treating a refractory metal.

40 A still further object of my invention is to provide a simple and inexpensive means for lowering the operating costs in the preparation of refractory metal bodies.

45 In order that my invention may be made readily apparent I shall describe the same with reference to the accompanying drawing wherein,

50 The single figure represents a somewhat dia-grammatical representation with some of the parts in elevation and others in cross section of the means illustrating my invention.

55 A device of the character generally employed in carrying out my invention may comprise a suitable yoke 10 supported by legs 11 resting on an appropriate foundation, not shown. United to said yoke is a base 12 having an insulating bushing 13 located therein. That side of the yoke opposite said base 12 also has an insulating bushing 14 located therein. Fixed to said bushing 14 so that the same is stationary with respect to said yoke is a contact terminal 15. The contact terminal 15 comprises a cylindrical portion 16 extending through an opening in said bushing and a flat plane faced disc 17 integral with the portion 16.

60 The contact 15, preferably composed of copper, may be provided with an insert 17' of tungsten, molybdenum or the like. The area of the face of the disc 17' is greater than the cross sectional area of the bar to be treated. A similar contact 18 is located in an opening through the bushing 13 and is adapted to move vertically in said bushing. Said bushing 13 has a recess 19 at one end thereof in which is located a compression spring 20 which surrounds the cylindrical

portion 21 of said contact and tends to force the same upwardly towards the relatively stationary contact 15.

65 Like the contact 15 the movable contact 18 also has a disc or insert 18' of the same characteristics as said disc 17'. A pair of conducting leads 23 and 24 have the respective ends thereof connected by means of a switch to the terminals of a suitable source of potential 25 and to contacts 15 and 18.

70 According to my invention the bar 26 to be treated is placed between the opposite faces of the contacts 15 and 18 with a sufficient quantity of loose tungsten powder 27 of the same general composition as that of the tungsten bar being located between the opposing faces of the contact terminals and the ends of the bar. This powder 27 preferably covers the entire surface of the ends of the bar 26 and may cover the entire surfaces of the contacts which I employ in this operation. 20

75 The depth of the tungsten powder 27, although variable, may generally be about  $\frac{1}{8}$  to  $\frac{1}{4}$  of an inch. After the bar is positioned in the manner heretofore set forth with tungsten powder located between the ends thereof and contact terminals 25 and, as illustrated in the drawing, an appropriate voltage is applied between the contacts 15 and 18 so that electric current may pass through the contacts, the powder and the tungsten bar. The magnitude of the current that passes through the bar and the time of so treating the bar are well known in the art and require no elucidation herein. It appears sufficient to say that the time of treatment and energy input are so regulated that the bar may be sufficiently heated in order to completely sinter the particles thereof. This heating operation is preferably done in a reducing atmosphere of hydrogen.

80 In the course of this treatment, in the manner heretofore set forth, the bar 26 itself has the particles thereof completely sintered and the particles of added powder 27 between the ends of the bar and the contact becomes at least partially sintered. At the end of the heat treating operation the bar may be readily removed from the contact terminals by a mere hand pulling operation. Generally, the bar so removed contains a partially sintered tungsten powder united thereto at the ends thereof. This layer of sintered powder at each end of the bar is somewhat fragile because the original tungsten powder at those places was comparatively loose. This sintered tungsten powder at each end of the bar may be readily removed therefrom by a mere rasping operation and when the bar so prepared is subjected to a rolling or mechanical operation generally followed in the preparation of tungsten wire, it is found very nearly one hundred percent of said bar is utilized in the preparation of the wire and there are no appreciable end losses. 60

85 Moreover, I have found that when this invention is employed the contact terminals have a relatively long life because they are not subjected to heavy arcing and, therefore, are not generally pitted, which pitting requires repairs or replacements.

90 Although I have described my invention with some particularity it is not to be limited thereby but is to be limited only by the prior art.

95 What is claimed is:

1. The method of treating a partially sintered bar which comprises locating said bar between a pair of contacts, placing a quantity of powdered tungsten between the outer ends of said bar and said contacts with said powder being contiguous 75

with substantially only the faces of said contact and the faces of said bar immediately adjacent each other, applying an electric potential between said contacts to elevate the temperature of said bar to further sinter the particles of said bar, maintaining said bar in position wholly by pressure exerted in the direction of the longitudinal axis of the bar.

2. The method of sintering a partially sintered tungsten bar whose mechanical strength is low,

comprising placing said bar between a pair of contacts, placing a quantity of tungsten powder substantially wholly between the transverse faces of said contacts and the transverse faces of said bar, and applying a potential between said contacts to substantially completely sinter said bar for greatly increasing the mechanical strength thereof.

THOMAS J. HANKINS, JR.

10